



US007431576B2

(12) **United States Patent**  
**Sun**

(10) **Patent No.:** **US 7,431,576 B2**  
(45) **Date of Patent:** **Oct. 7, 2008**

(54) **DUCTILE CAST IRON SCROLL  
COMPRESSOR**

(75) Inventor: **Zili Sun**, Arkadelphia, AR (US)

(73) Assignee: **Scroll Technologies**, Arkadelphia, AR  
(US)

(\*) Notice: Subject to any disclaimer, the term of this  
patent is extended or adjusted under 35  
U.S.C. 154(b) by 210 days.

(21) Appl. No.: **11/290,669**

(22) Filed: **Nov. 30, 2005**

(65) **Prior Publication Data**

US 2007/0122302 A1 May 31, 2007

(51) **Int. Cl.**

*F01C 21/00* (2006.01)  
*F01C 1/063* (2006.01)

(52) **U.S. Cl.** ..... **418/179; 418/55.2**

(58) **Field of Classification Search** ..... **418/55.1,  
418/178, 179, 152, 55.2**

See application file for complete search history.

(56) **References Cited**

U.S. PATENT DOCUMENTS

- 2,750,284 A \* 6/1956 Ihrig ..... 420/30  
3,055,756 A 9/1962 Kanter et al.  
3,421,886 A \* 1/1969 Schelleng ..... 420/22  
3,865,582 A \* 2/1975 Church et al. ..... 420/83  
4,363,661 A 12/1982 Kovacs  
4,944,663 A 7/1990 Iizuka et al.  
5,087,181 A \* 2/1992 Kamitsuma et al. ..... 418/178  
5,277,562 A \* 1/1994 Fukuhara et al. ..... 418/179  
5,439,360 A 8/1995 Barito  
5,478,417 A \* 12/1995 Heck et al. ..... 148/328  
5,548,973 A \* 8/1996 Komine et al. ..... 62/469  
5,580,230 A \* 12/1996 Keifer et al. ..... 418/55.5  
5,580,401 A 12/1996 Williamson  
5,755,271 A 5/1998 Williamson  
5,806,336 A 9/1998 Sunaga et al.

- 6,006,542 A 12/1999 Tojo et al.  
6,053,714 A 4/2000 Fenocchi et al.  
6,055,827 A 5/2000 Tojo et al.  
6,139,296 A 10/2000 Okajima et al.  
6,176,094 B1 1/2001 Ohta et al.  
6,189,322 B1 2/2001 Ishihara et al.  
6,286,334 B1 9/2001 Tojo et al.  
6,302,665 B1 10/2001 Esumi et al.  
RE37,520 E 1/2002 Williamson  
6,598,421 B1 7/2003 Suzuki et al.  
6,667,285 B1 12/2003 Kawahara et al.  
6,705,848 B2 \* 3/2004 Scancarello ..... 418/55.2

(Continued)

FOREIGN PATENT DOCUMENTS

EP 1331395 A2 7/2003

(Continued)

OTHER PUBLICATIONS

Metallurgy and Properties of Gray Irons, ASM Specialty Handbook,  
ASM International, 1996.

(Continued)

Primary Examiner—Thomas Denion

Assistant Examiner—Mary A Davis

(74) Attorney, Agent, or Firm—Carlson, Gaskey & Olds, PC

(57) **ABSTRACT**

A scroll compressor includes a scroll member having a base and a generally spiral wrap that extends from the base to define a portion of a compression chamber. The scroll member is made of a cast iron material comprising a microstructure having graphite nodules.

**13 Claims, 3 Drawing Sheets**



**U.S. PATENT DOCUMENTS**

6,860,315 B2 3/2005 Williamson  
6,874,325 B2 4/2005 Suzuki et al.  
6,948,922 B2 \* 9/2005 Esumi et al. .... 418/179  
7,265,080 B2 9/2007 Iso et al.  
2004/0140018 A1 \* 7/2004 Sato et al. .... 148/417  
2005/0210891 A1 9/2005 Matsumoto et al.  
2006/0191604 A1 \* 8/2006 Itoh et al. .... 148/321

**FOREIGN PATENT DOCUMENTS**

EP 1544469 6/2005  
EP 1652949 5/2006  
JP 59079089 5/1984  
JP 59079089 A \* 5/1984  
JP 9329091 12/1997

WO 2006072663 7/2006

**OTHER PUBLICATIONS**

Heat Treating of Gray irons, ASM Specialty Handbook, ASM International, 1996.

Standard Specification for Gray iron Castings, ASTM International.  
Standard Test Method for Evaluating the Microstructure of Graphite in Iron Castings, ASTM.

Ferrous Castings, Automotive Gray Iron Castings, SAE J431.

Standard Specification for Ductile Iron Castings, ASTM International.

Heat Treating of Ductile Irons, ASM Specialty Handbook, ASM International, 1996.

Metallurgy and Properties of Ductile Irons, ASM Specialty Handbook, ASM International, 1996.

Automotive Ductile (Nodular) Iron Castings, SAE J434 Feb. 2004.

European Search Report dated Sep. 14, 2007.

European Search Report dated Sep. 26, 2007.

\* cited by examiner



FIG.1





FIG.4



FIG.5



FIG.6



## DUCTILE CAST IRON SCROLL COMPRESSOR

## BACKGROUND OF THE INVENTION

This application relates to scroll compressors and, more particularly, to a scroll compressor member with improved strength and durability.

Scroll compressors are becoming widely utilized in refrigerant compression systems. As known, a pair of scroll members each has a base with a generally spiral wrap extending from the base. Typically, one scroll is non-orbiting and the other scroll orbits relative to the non-orbiting scroll. The orbiting scroll contacts the non-orbiting scroll to seal and define compression chambers. One of the two scroll members is caused to orbit relative to the other, with the size of the compression chambers decreasing toward a discharge port as refrigerant is being compressed.

One example refrigerant compression system includes an air conditioning or other environmental conditioning system. As is known, a compressor compresses a refrigerant and sends the refrigerant to a downstream heat exchanger, and typically a condenser. From the condenser, the refrigerant travels through a main expansion device, and then to an indoor heat exchanger, typically an evaporator. From the evaporator, the refrigerant returns to the compressor. Generally, the performance and efficiency of the system relies, at least in part, on the capacity and efficiency of the scroll compressor. Thus, there has been a trend toward higher capacity and higher efficiency scroll compressors.

One concern in designing higher capacity scroll compressors is the strength and durability of the scroll members. Higher capacity compressors operate under increasingly severe conditions, such as higher forces and increased wear between the scroll members. Use of current materials for the scroll members has proven successful in many compressors but may not be suited for more severe operating conditions. For example, under extreme operating conditions, the scroll members may break or wear excessively. Thus, even though higher capacity designs may be available, stronger and more durable scroll member materials are needed to realize the capacity benefits of such designs.

Accordingly, it would be desirable to provide scroll members that are able to withstand more severe conditions in order to enhance compressor capacity.

## SUMMARY OF THE INVENTION

One embodiment of a scroll compressor includes a scroll member having a base and a generally spiral wrap that extends from the base to define a portion of a compression chamber. The scroll member is made of a cast iron material comprising a microstructure having graphite nodules.

One embodiment scroll compressor includes a scroll member having a base and a generally spiral wrap that extends from the base to define a portion of a compression chamber. The scroll member is made of a material having a graphite nodule-forming agent.

One embodiment method of manufacturing the scroll compressor includes the steps of melting a cast iron material to produce a molten material, adding a nodule-forming agent to the molten material, and transferring the molten material into a mold having a shape of a scroll compressor member.

In the disclosed examples, the scroll member is relatively strong and durable. This allows the scroll compressor to withstand more severe operating conditions associated with high capacity compressor designs.

The above examples are not intended to be limiting. Additional examples are described below.

These and other features of the present invention can be best understood from the following specification and drawings, the following of which is a brief description.

## BRIEF DESCRIPTION OF THE DRAWINGS

FIG. 1 is a cross-sectional view of an example scroll compressor.

FIG. 2 is a perspective view of a non-orbiting scroll member for use in the scroll compressor of FIG. 1.

FIG. 3 is a perspective view of an orbiting scroll member for use in the scroll compressor of FIG. 1.

FIG. 4 is a schematic illustration of a microstructure having graphite nodules of a cast iron material used to make the scroll members.

FIG. 5 schematically illustrates another example microstructure having graphite nodules.

FIG. 6 schematically illustrates an example casting process.

## DETAILED DESCRIPTION OF THE PREFERRED EMBODIMENT

FIG. 1 shows a scroll compressor 20. As shown, a compressor pump set 22 is mounted within a sealed shell 24. A suction chamber 26 receives a suction refrigerant from a tube 28. As can be appreciated, this refrigerant can circulate within the chamber 26, and flows over an electric motor 28. The electric motor 28 drives a shaft 30 that defines an operative axis A for the compressor 20. The compressor pump set 22 includes a non-orbiting scroll 32 and an orbiting scroll 34. As is known, the shaft 30 drives the orbiting scroll 34 to orbit relative to the non-orbiting scroll 32.

FIG. 2 shows a perspective view of the non-orbiting scroll 32 and FIG. 3 shows a perspective view of the orbiting scroll 34. Each of the non-orbiting scroll 32 and orbiting scroll 34 includes a base portion 44 and a generally spiral wrap 46 that extends from the base portion 44. When assembled, the spiral wraps 46 interfit to define compression chamber 36 (FIG. 1) between the non-orbiting scroll 32 and orbiting scroll 34.

In the illustrated example, there is radial and axial compliance (relative to axis A) between the non-orbiting scroll 32 and orbiting scroll 34. Compliance allows the scrolls 32 and 34 to separate under certain conditions, such as to allow a particle to pass through the scroll compressor 20. Axial compliance maintains the wrap 46 of the orbiting scroll 34 in contact with the base portion 44 of the non-orbiting scroll 32 to provide a seal under normal operating conditions. A tap T taps a compressed refrigerant to a chamber 100 behind the base 44 of the orbiting scroll 34. The resultant force biases the two scroll members into contact. In other scroll compressors, the chamber can be behind the base of the non-orbiting scroll. Radial compliance maintains the wraps 46 of the non-orbiting scroll 32 and orbiting scroll 34 in contact under normal operating conditions.

Referring to FIG. 4, one or both of the non-orbiting scroll 32 and orbiting scroll 34 are made of a cast iron material having a microstructure 56 that includes graphite nodules 58. In the illustrated examples, the graphite nodules are within a matrix 60, such as a pearlite matrix. The microstructure 56 in this example is shown at a magnification of approximately 36x. The cast iron material is polished and etched in a known manner to reveal the microstructure 56.

The microstructure 56 includes an associated nodularity, which is a ratio of graphite nodules 58 to the total graphite

including other forms of graphite, within the matrix **60**. In one example, the nodularity is above about 80% and below 100%. In the example shown in FIG. 4, the nodularity is about 80%. In another example shown in FIG. 5, the nodularity is about 99%.

The graphite nodules **58** provide the non-orbiting scroll **32** and the orbiting scroll **34** with strength and durability. Other cast iron microstructures, such as those that include primarily graphite flakes, are weakened due to a notch effect at sharp edges of the graphite flakes. The graphite nodules **58**, however, are spheroidal in shape and therefore do not have the sharp edges that weaken the material. Generally, higher nodularity results in higher strength and higher toughness. In one example, the cast iron material with graphite nodules **58** has a tensile strength of at least 60 ksi. For example, the tensile strength can be tested using ASTM A395 or other known standard. The high strength and durability makes the non-orbiting scroll **32** and the orbiting scroll **34** relatively strong and wear resistant, which allows the scroll compressor **20** to be designed for relatively severe operating conditions and high capacities. In one example, use of cast iron material having graphite nodules **58** allows the wraps **46** to be increased in length (i.e., length extended from base **44**) to increase the size of the compression chambers **34** and, in turn, increase the capacity of the scroll compressor **20**.

In one example, the relatively severe operating conditions are caused, at least in part, from the axial and radial compliance between the non-orbiting scroll **32** and the orbiting scroll **34**. The axial and radial compliance causes contact between the non-orbiting scroll **32** and the orbiting scroll **34** as described above. During operation of the scroll compressor **20**, the contact causes wear and stress between the non-orbiting scroll **32** and the orbiting scroll **34**. The strong and durable cast iron material with graphite nodules **58** is suited to withstand such operating conditions.

The cast iron material of the non-orbiting scroll **32** and/or the orbiting scroll **34** includes a graphite nodule-forming agent that promotes formation of the graphite nodules **58** during casting. In one example, the cast iron material composition includes 3.20 wt %-4.10 wt % carbon, 1.80 wt %-3.00 wt % silicon, 0.10 wt %-1.00 wt % manganese, up to 0.050 wt % phosphorous, and an amount of the graphite nodule-forming agent. In a further example, the cast iron material composition includes about 3.60 wt %-3.80 wt % carbon.

In one example, the graphite nodule-forming agent includes magnesium. The magnesium is present in the cast iron material of the non-orbiting scroll **32** and/or the orbiting scroll **34** in an amount between about 0.02 wt % and about 0.08 wt %. In another example, the magnesium is present in an amount between about 0.03 wt % and about 0.06 wt %.

In another example, the graphite nodule-forming agent is an alloy, such as an alloy of magnesium. In one example, the alloy includes magnesium and nickel. The magnesium comprises between about 4 wt % and about 18 wt % of the alloy, the balance being nickel and possibly trace amounts of other materials.

In another example, the graphite nodule-forming agent includes both magnesium and cerium. In one example, the magnesium is present in the cast iron material of the non-orbiting scroll **32** and/or the orbiting scroll **34** in an amount as described above and the cerium is present in an amount between about 0.0005 wt % and about 0.01 wt %. The magnesium and cerium are added to the molten cast iron as described above. Alternatively, or in addition to magnesium and cerium, a rare earth metal is used in an amount up to 0.300 wt % to form the graphite nodules **58**. Example rare earth

metals include praseodymium, neodymium, promethium, samarium, europium, gadolinium, terbium, dysprosium, holmium, erbium, thulium, ytterbium, lutetium, yttrium, scandium, thorium, and zirconium, although use of these may be limited by availability and/or cost.

The graphite nodule-forming agent is added to molten cast iron during the casting process of the non-orbiting scroll **32** and/or the orbiting scroll **34**. For example, the amount added is suitable to result in the composition ranges described above.

The amount of graphite nodule-forming agent added to the molten cast iron is generally greater than the above-described composition ranges. In one example, about 0.3 wt % graphite nodule-forming agent is added. This provides the benefit of adding enough graphite nodule-forming agent to promote graphite nodule **58** formation while allowing for depletion of the graphite nodule-forming agent, such as through volatilization. Given this description, one of ordinary skill in the art will recognize suitable graphite nodule-forming agent amounts to add to the molten cast iron to meet their particular needs.

The amount of graphite nodule-forming agent controls the nodularity of the microstructure **56**. For example, a relatively small amount leads to lower nodularity and a relatively larger amount leads to a higher nodularity. Thus, the graphite nodule-forming agent composition ranges described herein can be used to tailor the properties, such as strength, wear, and galling, of the non-orbiting scroll **32** and/or the orbiting scroll **34** to the particular operational demands of the scroll compressor **20**.

FIG. 6 schematically illustrates an example casting process. A casting mold **70** defines a cavity **72** for forming the shape of the non-orbiting scroll **32** or orbiting scroll **34**. A container **74**, such as a ladle, holds molten cast iron material **76**, which will be poured into the casting mold **70** and solidify. Before pouring, a graphite nodule-forming agent **78** is added to the molten cast iron material **76**. Optionally, a predetermined period of time elapses between adding the graphite nodule-forming agent and pouring the molten cast iron material **76** into the casting mold **70** to allow dispersion of the graphite nodule-forming agent **78** in the molten cast iron material.

Although a preferred embodiment of this invention has been disclosed, a worker of ordinary skill in this art would recognize that certain modifications would come within the scope of this invention. For that reason, the following claims should be studied to determine the true scope and content of this invention.

What is claimed is:

1. A scroll compressor comprising:

a scroll member having a base and a generally spiral wrap that extends from said base to define at least a portion of a compression chamber, wherein said scroll member comprises a material having a 3.2 wt %-4.1 wt % carbon, 1.8 wt %-3 wt % silicon, 0.1 wt %-1 wt % manganese, about 0.02 wt %-0.08 wt % magnesium, about 0.0005 wt %-0.01 wt % cerium, about 0.3 wt % zirconium, and a balance of iron.

2. The scroll compressor as recited in claim 1, wherein the material includes a microstructure having graphite nodules.

3. The scroll compressor as recited in claim 2, wherein said graphite nodules are in a ferrite-pearlite matrix.

4. The scroll compressor as recited in claim 2, wherein said microstructure has a nodularity above about 80% and below 100%.

5. The scroll compressor as recited in claim 2, wherein said nodules are spheroidal.

6. The scroll compressor as recited in claim 1, including a second scroll member having a base and a generally spiral wrap extending from its base, said second scroll member being driven to orbit relative to said scroll member, said wraps of said scroll members inter-fitting to define said compression chamber, wherein said scroll members are axially and radially compliant.

7. The scroll compressor as recited in claim 1, wherein said magnesium comprises an alloy of nickel and said magnesium.

8. The scroll compressor as recited in claim 7, wherein said magnesium comprises between about 4 wt % and about 18 wt % of said alloy.

9. The scroll compressor as recited in claim 1, wherein said magnesium comprises between about 0.03 wt % and about 0.06 wt % of said material.

10. The scroll compressor as recited in claim 1, wherein said material has a tensile strength greater than 60 kpsi.

11. A method of manufacturing a scroll compressor, comprising:

5 (a) melting a cast iron material to produce a molten material;

(b) adding a nodule-forming agent to the molten material to form an alloy including 3.2 wt %-4.1 wt % carbon, 1.8 wt %-3 wt % silicon, 0.1 wt %-1 wt % manganese, about 0.02 wt %- 0.08 wt % magnesium, about 0.0005 wt %-0.01 wt % cerium, about 0.3 wt % zirconium, and a balance of iron; and

(c) transferring the molten material into a mold having a 10 shape to form a scroll compressor member.

12. The method as recited in claim 11, including cooling the molten material to form the scroll compressor member, including a base and a generally spiral wrap that extends from the base to define at least a portion of a compression chamber.

13. The method as recited in claim 11, including adding an 15 alloy of nickel and the magnesium.

\* \* \* \* \*

UNITED STATES PATENT AND TRADEMARK OFFICE  
**CERTIFICATE OF CORRECTION**

PATENT NO. : 7,431,576 B2  
APPLICATION NO. : 11/290669  
DATED : October 7, 2008  
INVENTOR(S) : Sun

Page 1 of 1

It is certified that error appears in the above-identified patent and that said Letters Patent is hereby corrected as shown below:

Claim 6, Column 5, line 1: "1" should read as --2--

Signed and Sealed this

Second Day of December, 2008



JON W. DUDAS  
*Director of the United States Patent and Trademark Office*